

March 10, 1959

3, 1959 O. ECKERT 2,877,183  
METHOD FOR IMPROVING THE MAGNETIC PROPERTIES OF FERRITE  
WITH A RECTANGULAR-SHAPED HYSTERESIS LOOP  
Filed March 6, 1956

Filed March 6, 1956

FIG. 1.



—FIG. 2.



FIG. 7



—FIG. 4—



INVENTOR.  
OSKAR ECKERT

BY  
Greene, Pinches & Durr

ATTORNEYS

1

2,877,183

## METHOD FOR IMPROVING THE MAGNETIC PROPERTIES OF FERRITE WITH A RECTANGULAR-SHAPED HYSTERESIS LOOP

Oskar Eckert, Lauf (Pegnitz), Germany, assignor to Steatit-Magnesia Aktiengesellschaft, Lauf (Pegnitz), Germany, a corporation of Germany

Application March 6, 1956, Serial No. 569,704

Claims priority, application Germany March 11, 1955

4 Claims. (Cl. 252—62.5)

Ferrites with a rectangularly-shaped hysteresis loop, hereafter referred to as rectangular ferrites, based on the double ferrite system  $x\text{MgO} \cdot y\text{MnO} \cdot z\text{Fe}_2\text{O}_3$ , have hitherto been known in the art. The application of such ferrites in electronical engineering, for example, as storage cores in the storage matrix of electronic calculators, is also familiar.

In such applications of rectangular ferrites for storage cores in electronic calculators, it is

(a) Desirable to achieve saturation with the lowest possible driving current; in relation to the loop shape, this means that the coercive force  $H_c$  should be as small as possible;

(b) To assure safe operation, it is a condition that the core in the state of, for example,  $-B_r$  when charged with a current pulse of  $+I$  and a magnetization pulse proportional thereto, changes its magnetization direction and switches to  $+B_r$ . However, in the condition of, for example  $-B_r$ , when charged with a current pulse of between  $+I$  and

$+I$   
2

corresponding to a magnetization impulse of between  $+H$  and

$+H$   
2

it should return to its condition of  $-B_r$ .

The above is more explicitly illustrated by means of the drawings.

Fig. 1 represents a hysteresis loop of a ring core ideally corresponding to the above conditions, while Fig. 2 represents the hysteresis loop of another ring core not satisfying the requirements. We charge both rings, each having a primary and a secondary winding on the primary side, with the pulse diagram sketched in Fig. 3 and, while the impulse magnitude is continually changing, examine in both cases the secondary voltage derived from the wave front of the positive pulse. The negative pulses which are scanned between the positive pulses, always force the core back to their condition  $-B_r$ . The secondary voltage as function of the magnetization field strength for both cases is shown in Fig. 4 (a) and (b).

This shows that this function in a core satisfying this condition shows a sharp breaking point for the secondary voltage, while the core not satisfying this condition shows a continuous rise of the secondary voltage, corresponding to the hysteresis loop, until saturation is reached. The wiring of the storage matrix requires that, for the clear distinction of working and disturb voltage, the disturb voltage in the limits of  $h=H/2$  may not amount to more than 5% of the secondary voltage  $U_{\max}$  delivered in the saturated condition, and a working voltage of 85% at a field strength of  $H$  of  $U_{\max}$  is sufficient. If one finds on the two curves the values corresponding to the 85% and 5%, respectively, of  $U_{\max}$  of  $H$ , and designates them  $H_2$  and  $H_1$ , the formulated requirement is equivalent to the statement that  $H_2:H_1 < 2$ . This requirement is ful-

2

filled for the first core of Fig. 1, while it is not true for the second core of Fig. 2.

Ferrites of the system  $\text{MgO} \cdot \text{MnO} \cdot \text{Fe}_2\text{O}_3$ , which show rectangular hysteresis loops, generally have a rather large coercive force of about 1.5–3 ampere windings/cm., and the requirement  $H_2:H_1 < 2$  can generally not always be fulfilled.

The invention relates to a magnesium-manganese ferrite with rectangularly shaped hysteresis loop and its object is the creation of an extended ferrite system of this type which permits the controllable regulation of the coercive force and of the relation  $H_2:H_1$ . In accordance with the invention, this is accomplished because the ferrite contains lead compounds.

According to a further development of the invention, such lead compounds are used in the raw mixtures which react in ceramic firing either directly or after decomposition with the iron oxide existing in the mixture, and form lead ferrite ( $\text{PbFe}_2\text{O}_4$ ).

In accordance with the invention, separately prepared lead ferrite, in quantities up to 10% of weight, calculated on the weight of the basic mixture, may be added to the pre-sintered basic mixture before the ceramic forming and firing.

25 The invention is illustrated by the following example.

By wet-ball milling, drying and firing, preferably between 850 and 1200° C., of a mixture of 35 mol percent  $\text{Fe}_2\text{O}_3$ , 35 mol percent  $\text{MnO}$  and 30 mol percent  $\text{MgO}$ , a ferrite powder is prepared. This is reground and ring cores are pressed therefrom according to ceramic production methods, whereupon the ring cores are subjected to a sintering fire at 1350°, and kept on this temperature for a period of two hours in normal atmosphere. The cores are dense and have the following properties:

|    |                      |                                                                       |                                    |
|----|----------------------|-----------------------------------------------------------------------|------------------------------------|
| 35 | Initial permeability | 40 . . . 60                                                           | oscillogr. absorption<br>at 50 Hz. |
|    | $B_r:B_s$            | 0.9                                                                   |                                    |
|    | $H_c$                | 1.6 aw./cm.                                                           |                                    |
| 40 | $H_2:H_1$            | 2.12 at $H_2=1.75$ amp. turns/cm.<br>by oscillogr. impulse measuring. |                                    |
|    | Curie temperature    | 300° C.                                                               |                                    |

In accordance with the invention, it has been shown that, when adding  $\text{PbFe}_2\text{O}_4$  in quantities up to <10% of weight of the above described basic mixture to this sintered basic mixture, the coercive force and the relation  $H_2:H_1$ , are improved without detriment to  $B_r:B_s$  value.

With the same production methods, one obtains the following properties:

| 50 | Basic mixture+weight percent $\text{PbFe}_2\text{O}_4$ | $\mu_0$ | $B_r:B_s$ | $H_c$ | $H_2:H_1$ | $T_c$ |
|----|--------------------------------------------------------|---------|-----------|-------|-----------|-------|
| 4  |                                                        | 40-60   | 0.9       | 1.19  | 1.77      | 300   |
| 6  |                                                        | 40-50   | 0.9       | 0.98  | 1.77      | 280   |
| 8  |                                                        | 40-50   | 0.87      | 0.88  | 1.78      | 270   |
| 55 | 10                                                     | 40-50   | 0.86      | 0.84  | 1.78      | 270   |

60 From these measurements, it is evident that the coercive force is considerably reduced, and that a ferrite, which, a priori, does not fulfill the conditions  $H_2:H_1 < 2$ , has yielded a ferrite which does fulfill such conditions and is safe for operation in electronic calculating machines, upon the addition of lead ferrite.

65 A further increase of the lead ferrite content impairs the rectangular shape of the hysteresis loop considerably and yields ferrites which are unsuited for the above described purposes.

In accordance with the invention, the production of the lead ferrite may be carried out jointly with the production of the other ferrite components in a simultaneous sinter-firing. It has been noted, however, that a greater consistency is assured when the lead ferrite is produced separately and added to the basic frit.

The mol percent of the magnesium oxide, manganese oxide and ferric oxide should be approximately as follows to obtain a square loop ferrite:

|                       | Mol percent      |
|-----------------------|------------------|
| Magnesium oxide ----- | 8 to about 55    |
| Manganese oxide ----- | 4 to about 66    |
| Ferric oxide -----    | 25 to about 47.5 |

The minimum addition of about 1% by weight of lead ferrite to the above ferrites is required to achieve the desired results in such compositions.

I claim:

1. A magnesium manganese ferrite at least 90-99% thereof consisting essentially of the components MnO, MgO and Fe<sub>2</sub>O<sub>3</sub>, the remaining 1-10% consisting of lead ferrite (PbFe<sub>2</sub>O<sub>4</sub>).

2. The ferrite as claimed in claim 1 wherein the MnO, MgO and Fe<sub>2</sub>O<sub>3</sub> components are present in the proportion of about 35 mol proportion of MnO, about 30 mol proportions of MgO and about 35 mol proportions of Fe<sub>2</sub>O<sub>3</sub>.

3. In a process making a manganese-magnesium-ferrite with a square hysteresis loop comprising mixing the

manganese oxide, magnesium oxide and ferric oxide components in proportions to provide a square loop ferrite and adding a lead-oxygen compound to said mixture in proportions to form 1 to 10% by weight of PbFe<sub>2</sub>O<sub>4</sub> in the resultant product and thereafter firing said mix to produce the ferrite compound.

4. In a process as claimed in claim 3 comprising pre-forming a lead ferrite of the formula PbFe<sub>2</sub>O<sub>4</sub> and adding this compound to the mixture of MgO, MnO and Fe<sub>2</sub>O<sub>3</sub> as the lead-oxygen compound.

#### References Cited in the file of this patent

##### UNITED STATES PATENTS

15 2,736,708 Crowley ----- Feb. 28, 1956

##### FOREIGN PATENTS

5 516,395 Belgium ----- June 19, 1953  
735,375 Great Britain ----- Aug. 17, 1955

##### OTHER REFERENCES

20 "Arkin for Kemi, Mineralogi Och." Band 12A, No. 29, pages 1-9, 1938.